

## UNITED STATES PATENT OFFICE

VIGGO DREWSSEN, OF LARCHMONT, NEW YORK, ASSIGNOR TO WEST VIRGINIA PULP  
AND PAPER COMPANY, OF NEW YORK, N. Y., A CORPORATION OF DELAWARE

## METHOD FOR RECOVERY OF ROSIN SOAP MATERIAL FROM SPENT WOOD LIQUORS

No Drawing.

Application filed January 11, 1928. Serial No. 246,095.

This invention relates to the recovery of a rosin soap material from spent liquors resulting from the cooking of coniferous woods for the manufacture of paper pulp or other purposes.

When coniferous woods are cooked with alkaline liquors or with sodium monosulphite liquors, rosin and fatty acids in the wood are saponified and become incorporated in the liquor. Again, when coniferous woods are cooked with acid cooking liquors, rosins and fats may be emulsified and incorporated in the liquor so that when the spent liquor is neutralized with caustic alkali (a practice frequently resorted to in order to treat the spent liquor in iron apparatus without corrosion) similar soaps are formed in the liquor.

If the liquor is concentrated, the soaps may be salted out of the liquor and if suitably concentrated liquor is allowed to stand and cool sufficiently, the soaps will collect as a scum at the top. In the practice, however, cooling and settling of the concentrated spent liquor sufficiently to recover good yields of the soapy content is uneconomical since it wastefully dissipates heat that can be used advantageously in further treating the liquor for recovery of chemicals therein or in the preparation thereof for burning. Moreover, the removal of the soap from the settling apparatus involves laborious time-consuming work. The formation of soap scums in the later stages of the evaporators in which spent liquors are commonly concentrated is generally regarded in the industry as a costly nuisance necessitating frequent cleaning of the evaporators rather than as the source of a valuable by-product. Ordinarily the evaporators and particularly the third and fourth effects have to be cleaned weekly to remove soap scums. Moreover, after each cleaning the efficiency of the evaporators again falls off continuously due to the accumulation of thicker and thicker soap scums.

Various methods for recovering soapy materials from such spent liquors have heretofore been suggested but none of them have proven satisfactory.

According to the present invention, the spent liquor may be passed continuously through a centrifugal separator whereby the soapy materials are continuously removed and flow to suitable soap vats and the soap-free liquor returned to the concentrating system. The separating machine may advantageously be of the type commonly used for separating cream from milk or of the type commonly used for separating water from oil. It is important to have the liquor at a proper concentration and temperature at the time when it is run into the separating machine. Concentration of the spent liquor automatically effects a gradual salting out of the soapy constituents therein. The salting out action is also increased as the temperature of the liquor falls. Temperatures below 60° C. are usually needed for good yields. The temperature should be high enough, however, so that the soap can be freely flowed through the separating machine and it is desirable to avoid temperatures so low as to deposit soap in the evaporators prior to the sending of the liquor to the separating machine. Usually the temperature should be above 25° C. The liquor at the time of treatment may advantageously be of such concentration and temperature that the soapy materials salted out of the spent liquor are largely dispersed throughout the liquor in tiny liquid globules like cream in milk. The concentration must be carried to a stage at which the gravity of the liquid is materially different from the gravity of the soapy materials. For example, when the specific gravity of the soap is about 1.05, the spent liquor should be evaporated to a specific gravity between about 1.1 and 1.15; on the other hand, with a soap having a gravity of 1.13 a good separation has been accomplished with a liquor of 1.10, the flow of separated soap and liquor being reversed. The optimum specific gravity and temperature for the liquor entering the machine vary somewhat with different liquors, depending particularly upon the ratio of salts to soaps therein contained and the gravity and solubility of the soap. Optimum conditions for a particular plant and liquor may readily be deter-

100

mined in accordance with the foregoing principles as indicated by the following example.

A certain spent liquor was subjected to evaporation in a series of multiple effect evaporators in accordance with standard practice. The liquor, as delivered to the evaporator and as it existed after passage through one effect of the evaporator, was found to be too dilute to yield substantial separation if passed through a centrifugal machine. After passing through two effects of the evaporator, the liquor was approximately halved in volume and consequently doubled in concentration so that it then approximated a specific gravity of 1.10. The salts dissolved in the spent liquor had by this time become sufficiently concentrated to effect at the temperature prevailing in the evaporator an automatic salting out of a substantial portion of the dissolved soap in the form of tiny globules almost colloidally dispersed throughout the spent liquor. The existence of the separated globules was, of course, invisible to the eye in the black liquor just as the cream is invisible in fresh milk. It was found convenient to test the extent of the salting out of the soap in the liquor at each stage by whirling a small sample in an ordinary Babcock milk testing centrifuge.

The indications afforded by the Babcock machine in this instance were confirmed by passing the liquor from the second effect through a De Laval or a Sharpless separator at different temperatures. Practically no separation of soap occurred at temperatures of 70° C. or over. About 3 lbs. per 100 gals. was recovered at 60° C., about 5.8 lbs. per 100 gals. at 50° C., about 6.5 lbs. per 100 gals. at 45° C., and about 7.4 lbs. per 100 gals. at 42° C. This was about as cool as it seemed desirable to cool the liquor although slightly greater recoveries were obtained by continuing the cooling down to 25° C.

It was found that liquor taken after passing through three effects of the evaporator had become too concentrated for treatment in the centrifugal machine as it yielded only one and a half pounds per 100 gals., the reason being that most of the soap had already separated out and been deposited in the third effect of the evaporator. For this particular plant and type of liquor, therefore, it seemed desirable to take the liquor from the second stage of the evaporator. The temperature of liquor from the second evaporator averaged about 45° C. but was subject to fluctuations. It was found desirable to provide means for keeping its temperature uniform at about 45° C.

It was found desirable to warm the discharge passage for the soap from the separating machine so as to prevent congealing of the soap on the walls and gradual contraction of the passage.

The soap material, which flowed from the separator, was practically free from residual liquor. It yielded a clear amber colored solution with water. A typical sample had a specific gravity of about 1.049 and contained about 36% of rosin acids and 23% of fatty acids and about 34% moisture. The total alkali computed as Na<sub>2</sub>O was about 4.37. This soapy mixture makes an excellent size. It is also useful as a soap stock.

It will be obvious from the foregoing that the method and process may be modified in many details without departing from the spirit and scope of my invention.

What I claim is:

1. A method of recovering soaps dissolved in spent wood treating liquor which comprises concentrating the liquor to a specific gravity of approximately 1.1 to 1.15, and at which the gravity of the liquor differs from the gravity of the soap, and subjecting such liquor at a temperature between about 25 to 60 degrees centigrade to centrifugal separation.

2. A process for the recovery of soap from spent wood treating liquors which comprises evaporating the spent liquors to a concentration whereat the gravity of the liquor differs from the gravity of the soap therein, subjecting such concentrated liquor at a temperature at which the soap is largely dispersed through the liquor in minute globules to centrifugal separation and collecting said soap.

3. A process for the recovery of soap from spent wood treating liquors, which comprises concentrating the liquor until the specific gravity of the liquor differs from the specific gravity of the soapy constituents therein and soapy constituents have been salted out, subjecting such concentrated liquor to centrifugal separation and collecting said soap.

4. A process for the recovery of soaps from spent wood treating liquors, which comprises concentrating the liquor until the specific gravity of the liquor differs from the specific gravity of the soapy constituents therein and soapy constituents have been salted out, subjecting such concentrated liquor to centrifugal separation at a temperature between 25° C. and 60° C., and collecting said soap.

5. A continuous process for the treatment of spent wood treating liquors containing soap which comprises evaporating the spent liquors to a concentration whereat the gravity of the liquor differs from the gravity of the soap therein, subjecting such concentrated liquor to centrifugal separation at a temperature at which the soap is largely dispersed through the liquor in minute globules, collecting the soap, and returning the separated liquor for further concentration.

6. A continuous process for the treatment of spent wood treating liquors containing soap which comprises concentrating the liquor until the specific gravity thereof differs

from the specific gravity of the soapy constituents therein and soapy constituents have been salted out, subjecting such concentrated liquor to centrifugal separation at a temperature between 25° C. and 60° C., collecting the soap, and returning the separated liquor for further concentration.

5 In testimony whereof, I have signed my name to this specification this 9th day of  
10 January, 1928.

VIGGO DREWSEN.

15

20

25

30

35

40

45

50

55

60

65